

## 1

2,999,067

## SYNTHETIC OIL ADDITIVE

Thomas F. Banigan, Jr., Walnut Creek, Calif., assignor to Tidewater Oil Company, San Francisco, Calif., a corporation of Delaware

No Drawing. Filed Nov. 27, 1956, Ser. No. 624,498  
9 Claims. (Cl. 252—49.8)

This invention relates to a new family of chemical compounds comprising a group of linear polymeric esters, particularly useful as viscosity-index improvers for certain types of synthetic lubricating oils. The invention also relates to synthetic lubricating oil chosen from the group consisting of the diesters and the phosphate esters having an improved viscosity index as a result of addition of compounds of this invention. The invention further relates to a method for producing the new family of compounds and to a method for improving the viscosity indices of certain synthetic ester lubricating oils.

In recent years synthetic lubricants have been developed in an attempt to meet the stringent requirements of new engines, including jet aircraft engines. These are superior to hydrocarbon oils in their ability to withstand temperatures as high as 450° F. without breaking down. They also flow at —65° F. and possess numerous other qualities enabling them to perform well under difficult conditions.

One class of such synthetic lubricating oil is usually referred to as "diesters." Examples are the (2-ethylhexyl) diesters, such as dioctyl azelate, dioctyl sebacate, dioctyl glutarate, and dioctyl adipate. In addition there are various sebacates such as di-(methylethyl) sebacate, di-(3-methylbutyl) sebacate, di-(2-ethylbutyl) sebacate, di-(1,3-dimethylbutyl) sebacate, di(undecyl) sebacate, di(tetradecyl) sebacate, and di(heptadecyl) sebacate. There are corresponding adipates, azelates, and glutarates. There are other diesters such as 1,6-hexamethylene glycol di-(2-ethylhexanoate), tri-ethylene glycol di-(2-ethylhexanoate), and di-[2-(2'-butoxyethoxy)ethyl]adipate. There are also useful phthalate diesters, such as dibutyl phthalate (di-n-butyl orthophthalate). All these compounds may be grouped as diester synthetic lubricating oils, or aliphatic branched-chain diesters that remain liquid in the temperature range from about —30° F. to 300° F.

Another type of synthetic oil to which this invention relates comprises the phosphate esters such as tributyl phosphate and tricresyl phosphate.

The diester synthetic lubricating oils as a class possess high viscosity indices. However, some of the lower-molecular-weight members such as dioctyl adipate tend to be relatively deficient in this property, thus eliminating them from consideration as jet engine lubricants. It is the lower-molecular-weight diesters which offer the greatest promise for the future development of lubricants which will remain fluid at extremely low temperatures. The phosphate esters have outstanding lubricity characteristics, excelling most other classes of synthetic oils. Low viscosity index is probably the chief obstacle to their wider use as specialty lubricants. It has therefore been a problem to produce an additive which would increase the viscosity index in these two groups of synthetic oils, without causing trouble elsewhere. To do so is one of the objects of this invention, which accomplishes it by means of a new family of chemical compounds.

Another object of the invention is to provide a viscosity index improver such that the improvement takes place when only a small quantity of the improver is added, thereby not interfering with the other qualities of the synthetic lubricant and holding costs down.

## 2

*The new compound broadly*

The new compounds of the present invention comprise a new class of linear polymeric esters, the class being defined by the general formula:



in which

10 G represents a polypropylene glycol group of at least 7 alkylene radicals joined linearly by ether oxygen atoms;

A represents an organic dibasic acid radical;

n is a number lying between 0.875 and 1.111;

15 x is an integer corresponding to the average degree of polymerization; and

R<sub>1</sub> and R<sub>2</sub> each represent an end group either or both of which may be a hydroxy radical, a carboxy radical, or an alkyl or aryl group.

The chemical nature of the end groups R<sub>1</sub> and R<sub>2</sub>, with 20 respect to the functioning of these polymers as viscosity index improvers, appears secondary in importance to several other factors, including: (a) the molecular weight of the polypropylene glycol, (b) the dibasic acid used, and (c) the degree of polymerization. However, there have 25 been indications that the introduction of relatively non-polar end groups helps to protect the polymer from haze and color formation during preparation and is therefore preferable to the hydroxy and carboxy end groups.

*The polypropylene glycol group (G)*

30 Polymers prepared from polyoxyalkylene glycols composed of alkylene radicals of less than 3 carbon atoms, such as polyethylene glycols, usually proved to be water soluble and were invariably insoluble in the synthetic 35 lubricating oils disclosed herein.

However, polymers prepared from polypropylene glycols have displayed the requisite solubility in the synthetic 40 lubricating oils when said polypropylene glycols contained 7 or more oxypropylene units. Optimum activity 45 as a viscosity-index improver was noted with a polymer prepared from polypropylene glycol possessing 35 oxypropylene units. Only slightly less effective was the polymer made from a glycol with 17 oxypropylene units. Still soluble in synthetic lubricants, but much less effective, was the polymer made using a glycol with 8 oxypropylene units. The use of tripropylene glycol (3 oxypropylene units) gave rise to an insoluble polymer. The 50 tests indicate that there should be at least 7 oxypropylene groups, and there may be as many as 35 or 40.

*The dibasic acid radical (A)*

Various dibasic organic acids may be used. Excellent 55 results are obtained where A is the oxayl radical, but carbonyl, succinyl, adipyl, sebacyl, isophthalyl, orthophthalyl, and terephthalyl radicals have also given good compounds.

Polymers prepared by reaction of polypropylene glycols 60 (containing 7 or more oxypropylene units) with dibasic acid chlorides (see the description of the method) ranging from oxalic to sebacyl have all been shown to be soluble in the synthetic oils claimed herein. However, the polymers prepared using oxayl chloride have invariably been the most potent viscosity index improvers as well as possessing the least color and haze. The somewhat greater reactivity of oxayl chloride compared to the higher acid chlorides enables the use of lower reaction temperatures, a condition which favors the production of a very high polymer possessing a minimum 65 of color and haze.

*The ratio of glycol to dibasic acid (G/A or n)*

Optimum results are usually obtained where equimolar ratios of glycol and acid halide are used. This favors a high degree of polymerization yielding a polymer with

However, the use of non-polar end groups, those in (4) above, does give more clarity and freedom from haze and color formation. Typical compounds are shown in Table I below.

TABLE I  
*Chemical composition of synthetic polyoxypropylene esters*

| Polymer | R <sub>1</sub>                             | R <sub>2</sub>                             | A             | G •     | Viscosities b | G/A • |
|---------|--------------------------------------------|--------------------------------------------|---------------|---------|---------------|-------|
| #1      | hydroxy                                    | hydroxy                                    | terephthalyl  | PPG1025 | 300           | 1.111 |
| #2      | do                                         | do                                         | orthophthalyl | PPG1025 | 475           | 1.111 |
| #3      | polypropylene glycol ether 65 <sup>d</sup> | polypropylene glycol ether 65 <sup>d</sup> | do            | PPG1025 | 1,500         | 0.875 |
| #4      | hydroxy                                    | carboxy                                    | oxaryl        | PPG2025 | 1,200         | 1.000 |
| #5      | n-butyl                                    | n-butyl                                    | do            | PPG2025 | 60,000        | 0.875 |
| #6      | do                                         | do                                         | do            | TPG     | 5,000         | 0.950 |
| #7      | do                                         | do                                         | do            | PPG1025 | 20,000        | 0.875 |
| #8      | hydroxy                                    | carboxy                                    | adipyl        | PPG2025 | 4,200         | 1.000 |

<sup>a</sup> PPG = polypropylene glycol, TPG = tripropylene glycol, and the numbers refer to the average molecular weight, from which number of oxyalkylene units can be calculated.

<sup>b</sup> Viscosities at 210° F. in seconds Saybolt Universal are a function of chain length.

<sup>c</sup> G/A refers to the ratio of glycol to dibasic acid.

<sup>d</sup> Sold commercially by Carbide and Carbon Chemical Company under the trade-name of Ucon LB-65, the 65 referring to the Saybolt Universal viscosity at 100° F.

great capacity for improving the viscosity index of certain synthetic oils. Polymers useful for this purpose can be obtained where the glycol to acid halide ratio lies within the range 0.875 to 1.111 and with end groups R<sub>1</sub> and R<sub>2</sub> from any of the four choices enumerated below.

*The degree of polymerization (x)*

It is difficult to determine x precisely because of the rather high molecular weight of the polymers; moreover, x appears to be capable of variation over wide limits depending on the molecular weight of the oxyalkylene glycol used in the polymerization. A smaller x can give a useful polymer when a high molecular weight glycol is used such as polypropylene glycol 2025 (a propylene glycol polymer having an average molecular weight of 2025) whereas a larger x is needed for a lower molecular weight glycol. Viscosity has been found useful as a guide to the required molecular weight. For example, polymers ranging in viscosity (210° F.) from about 250 to 13,000 centistokes, and especially those from about 4000 to 13,000 centistokes, have shown activity as viscosity index improvers. Polymers of this same type with even higher viscosities should also prove useful if they possess the requisite solubility and shear stability characteristics (extremely high molecular weight polymers are often deficient in such properties).

*The end groups R<sub>1</sub> and R<sub>2</sub>*

R<sub>1</sub> and R<sub>2</sub> will generally be:

- (1) An hydroxy radical in both cases if excess polyoxyalkylene glycol was used in preparation,
- (2) A carboxy radical in both cases if excess dibasic acid was used,
- (3) One hydroxy and one carboxy radical, respectively, if equimolar reagent ratios were used, or

(4) An alkyl or aryl group, if excess dibasic acid dihalide is used to produce a polymer possessing terminal acyl halide atoms capable of further condensation reaction as with an alcohol or phenol, such as methanol, ethanol, n-butanol, ethylene glycol monoethyl ether, diethylene glycol mono-n-butyl ether, polypropylene glycol monomethyl ether, tripropylene glycol mono-n-butyl ether, polypropylene glycol 425 mono-n-butyl ether, phenol, paracresol, and nonylphenol.

As stated earlier, the end groups R<sub>1</sub> and R<sub>2</sub> are relatively unimportant, merely a necessary chemical fact.

Some important qualities of each of these compounds are shown in Table II, the number assigned each polymer remaining the same through all tables and examples in this specification.

TABLE II  
*Analytical data of synthetic polymers*

| Polymer | Acid No. <sup>a</sup> | Sap. No. <sup>b</sup> | Vis. @ 210 (SSU) <sup>c</sup> | Color (ASTM) <sup>d</sup> |
|---------|-----------------------|-----------------------|-------------------------------|---------------------------|
| #1      | 0.13                  | 76                    | 300                           | 1                         |
| #2      | 12                    | 92                    | 475                           | 1+                        |
| #3      | 11                    | 104                   | 1,500                         | 1+                        |
| #4      | 8                     | 39                    | 1,200                         | 1-                        |
| #5      | 12                    | 59                    | 60,000                        | 1                         |
| #6      | 113                   | 459                   | 5,000                         | 1½                        |
| #7      | 26                    | 118                   | 20,000                        | 2½                        |
| #8      | 1.8                   | 56                    | 4,200                         | 2                         |

<sup>a</sup> Acid No.—as in ASTM-D974-55T.

<sup>b</sup> Saponification No. as in ASTM-D94-55T.

<sup>c</sup> Viscosities at 210° in Saybolt Seconds Universal.

<sup>d</sup> Color—ASTM-D-155-45T.

*Methods of preparing the polypropylene esters*

Two preferred methods of preparation may be used: (1) ester exchange and (2) reaction of glycols with dibasic acid dichlorides. The second method is an excellent one for research work, with high yields of high molecular weight polymers with minimum effort, while the first method uses cheaper and less reactive intermediates and is therefore better suited to commercial manufacture. Examples of each type follow.

The two preferred methods are aspects or embodiments of a single broad concept, namely, that of reacting polypropylene glycol with a dibasic acid derivative. The derivative is preferably chosen from the group consisting of the dibasic acid diesters and the dibasic acid dichlorides.

*FIRST METHOD: ESTER EXCHANGE*

When the dibasic acid diester is used in the method of preparing these polypropylene glycol esters, the reaction takes place in the presence of a basic catalyst, such as sodium methylate. Preferably, the reaction is conducted in an inert atmosphere, heat being applied so that the temperatures lie in the range between 150° C. and 200° C. Methyl alcohol is formed as a by-product but may easily be removed. Preferably, the reagents are diluted with some suitable solvent, such as xylene, to prevent sublimation of the dibasic acid diester. The following example of the first method (ester exchange) follows.

5

*Example 1.—Preparation of poly [polypropylene glycol 1025 (10)—terephthalate (9)] (polymer #1) by ester exchange*

| Reagents                                          | Wt.,<br>grams | Moles |
|---------------------------------------------------|---------------|-------|
| Polypropylene glycol 1025 (molecular weight 1025) | 293           | 0.286 |
| Dimethyl terephthalate                            | 50            | 0.257 |
| Sodium methylate (catalyst)                       | 5             |       |

The reaction was conducted in a 1-liter, 3-necked, round-bottomed flask equipped with a stirrer, a thermometer and a condenser with water trap, and provided with a nitrogen atmosphere. The reagents proved to be miscible at about 100° C. but further heat caused the terephthalate to sublime. Therefore, the contents were cooled, diluted with 100 ml. of xylene, mixed with 5 g. of sodium methylate, and heated slowly to 170-175° C. After three hours of refluxing 19.5 ml. of methanol was removed azeotropically. Vacuum was then applied and the temperature raised gradually to 200° C. to remove the solvent and force the reaction toward completion. The product was obtained as 317 g. (97% theor.) of a straw colored resin. The crude polymer was purified by dilution with three parts of pentane, followed by charcoal and clay treatment and filtration. On evaporation of the pentane from the filtrate the polymer was obtained as 291 g. of very pale viscous oil.

The polymer exhibited the properties tabulated in Tables I and II under polymer #1. Also it had a refractive index  $n_{D^{20}}$  of 1.4664 and a specific gravity (sp. gr.<sub>20</sub><sup>20</sup>) of 1.04.

## SECOND METHOD: REACTION OF GLYCOLS WITH DIBASIC ACID DICHLORIDE

Broadly speaking, the second method, that of reaction of glycols with dibasic acid dichlorides, is carried on in the presence of an acid acceptor, such as pyridine or tributyl amine. Since the dichloride radical is the one to be removed, a still more accurate designation of the acid acceptor would be to say that it is an HCl acceptor. This reaction also forms a by-product, the hydrochloride of the HCl acceptor, such as pyridine hydrochloride.

This reaction does not require a high temperature, and in fact may take place at low temperatures, around 5° to 10° C. To insure completion of the reaction, the temperature may be gradually increased up to about as high as 85° or 90° C.—less than 100° C. It has been found preferable, though not essential, when using this method, to remove all the water by means of a trap prior to the halide addition, because such removal gives rise to a higher degree of polymerization. The following examples illustrate this second method.

Example 2.—Preparation of poly[polypropylene glycol 1025 (7)-orthophthalate (8)-polypropylene glycol ether 65 (2)] (polymer #3) by reaction of glycol with dibasic acid dichloride

| Reagents                        | Wt.,<br>grams | Moles |
|---------------------------------|---------------|-------|
| Polypropylene glycol 1025.....  | 300           | 0.292 |
| Orthophthalyl chloride.....     | 67            | 0.330 |
| Polypropylene glycol ether..... | 32            | 0.073 |
| Pyridine.....                   | 65            | 0.320 |

Another way of stating the formula of this composition is



where  $m$  is about 3 and  $n$  is about 17.

6

The orthophthalyl chloride diluted with an equal volume of benzene was added dropwise to a stirred solution of the glycol and 47 g. of pyridine dissolved in 100 ml. of dry benzene. The temperature was held at 10° C. by external cooling. Reaction was indicated by copious salt formation (pyridine hydrochloride). The polypropylene glycol ether (Carbon and Carbide Chemical Company Ucon LB-65) was mixed with 18 g. of pyridine and 50 ml. of benzene and was introduced dropwise after the chloride was in. The reaction mixture was diluted with additional benzene and stirred for about three hours at temperatures of 25-45° C. The polymer solution was then filtered from the by-product pyridine hydrochloride, decolorized with charcoal and super cel, refiltered, and solvent-evaporated to give 352 g. of yellow viscous resin.

In addition to the properties given in Tables I and II, the following properties were found for polymer #3: Refractive index  $n_D^{20}$  of 1.4689, viscosity at 130° F. of 6875 Saybolt Universal Seconds, and a viscosity index of 124.

*Example 3.—Preparation of Poly[polypropylene glycol 2025 (1)-oxalate(1)] (polymer #4) by reaction of glycol with dibasic acid dichloride*

|    | Reagents                  | Wt.,<br>grams | Moles |
|----|---------------------------|---------------|-------|
| 30 |                           |               |       |
|    | Polypropylene glycol 2025 | 300           | 0.146 |
|    | Oxalyl chloride           | 18.5          | 0.146 |
|    | Pyridine                  | 25            | 0.316 |

The glycol, molecular weight of 2025, and pyridine were mixed together with 150 ml. of dry benzene, placed in a reaction flask and cooled to 5° C. The oxalyl chloride in an equal volume of benzene was then added drop-wise during one hour to the stirred reaction mixture held at 5–10° C. An additional 50 ml. of benzene was added, and stirring continued as the temperature was gradually raised to about 85° C. The reaction mixture was refluxed for three hours and allowed to stand overnight. The product was thinned with additional benzene and filtered to remove pyridine hydrochloride. The solvents were removed under vacuum with the aid of a nitrogen bubbler to yield 290 g. (94% theor.) of virtually colorless viscous resin.

In addition to the properties noted in Tables I and II, the refractive index  $n_D^{20}$  was 1.4522.

55

*Example 4.—Preparation of poly[polypropylene glycol 2025 (7)-oxalate(8)-n-butyl(2)] (polymer #5) by reaction of the glycol with the dibasic acid dichloride and with n-butyl end groups added*

|    | Reagents                       | Wt.,<br>grams | Moles |
|----|--------------------------------|---------------|-------|
| 65 | Polypropylene glycol 2025..... | 300           | 0.148 |
|    | Oxalyl chloride.....           | 21.5          | 0.169 |
|    | n-Butyl alcohol.....           | 12            | 0.16  |
|    | Pyridine.....                  | 37            | 0.47  |

Another way of expressing the formula of this 5 composition is



wherein  $n$  averages about 34.

The reaction was conducted essentially according to directions outlined for the preparation of polymer #5.

The glycol, pyridine and 200 ml. of benzene were refluxed until a total of 0.5 ml. of water had been removed by means of a trap. (This exhaustive removal of water gave rise to a higher degree of polymerization than in Example 3.) The oxalyl chloride in benzene was added dropwise to the cooled, stirred solution as before. Extreme viscosity of the reaction mixture necessitated several dilutions with benzene during the reaction period. The temperature was gradually elevated to 85° C. and then cooled to 40° C. At this point a mixture of n-butyl alcohol and pyridine was added dropwise. Stirring was continued and the contents allowed to stand overnight. The mixture was diluted with 750 ml. of n-heptane and filtered. The filtrate was charcoal treated, filtered and solvent-evaporated to yield 301 g. (95% theor.) of extremely viscous pale yellow resin.

Example 5.—Preparation of poly[tripropylene glycol (19)-oxalate(20)-n-butyl (2)] (polymer #6) by the method of Example #4

| Reagents                 | Wt.,<br>grams | Moles |
|--------------------------|---------------|-------|
| Tripropylene glycol..... | 86            | 0.450 |
| Oxalyl chloride.....     | 60            | 0.472 |
| n-Butyl alcohol.....     | 12            | 0.162 |
| Pyridine.....            | 85            | 1.08  |

This reaction was conducted according to the directions outlined for the preparation of polymer #5. All traces of water were removed by azeotropic distillation as before. The polymer was obtained as 99 g. (97% yield) of a very viscous light amber resin.

*Example 6.—Preparation of poly[polypropylene glycol 1025 (7)-oxalate(8)-n-butyl (2)] (polymer #7) by the method of Example #4*

| Reagents                       | Wt.,<br>grams | Moles |
|--------------------------------|---------------|-------|
| Polypropylene glycol 1025..... | 150           | 0.146 |
| Oxalyl chloride.....           | 21.2          | 0.167 |
| <i>n</i> -Butyl alcohol.....   | 12            | 0.162 |
| Pyridine.....                  | 36.5          | 0.461 |

This reaction was carried out according to directions for polymer #5 with special care again directed to trace water removal. The polymer was obtained as 158 g. (99.5% theor.) of very viscous light brown resin.

*Example 7.—Preparation of poly[polypropylene glycol 2025 (1)-adipate(1)] (polymer #8) by the method of Example #4.*

| Reagents                       | Wt.,<br>grams | Moles |
|--------------------------------|---------------|-------|
| Polypropylene glycol 2025----- | 300           | 0.148 |
| Adipyl chloride-----           | 27.1          | 0.148 |
| Pyridine-----                  | 25            | 0.320 |

15 Pyridine hydrochloride (by-product) formed copiously at the initial reaction temperature of 10° C. As the solution viscosity remained low compared to earlier preparations of oxalate polyesters, external heat was applied to force the reaction. A reaction temperature of 85° C.  
20 was held for about 3.5 hours following addition of the adipyl chloride to the stirred glycol-benzene-pyridine solution. No noticeable increase in solution viscosity occurred after about three hours of refluxing. The product resin was isolated as before to yield 309 g. (98% theor.) of viscous straw-colored polymer. This resin showed a greater tendency toward mineral oil solubility than did corresponding oxalates. However, it is still deficient in this property.  
25

30 *Use of the polymers of this invention as viscosity index improvers*

Representative polymers of this invention were evaluated as viscosity index improvers in various mineral oil stocks and in four of the principal classes of synthetic lubricating oils including (a) diesters, (b) polyglycol ethers, (c) silicones, and (d) phosphorous compounds. The first thing tested was their solubility in the various oils, shown in Table III.

As Table III shows, these polymers had only limited solubility in the mineral oil stocks including both solvent pale and bright stocks, so they could not be used therein. They appeared to be completely insoluble and hence without effect on the silicone oils tested. The polymers were entirely miscible with the polyglycol ethers but later research showed that they had no effect on the viscosity-temperature characteristics of this class of synthetic oils.

The new polymers were very soluble in the diester oils and exhibited high viscosity index activity, comparable and often better than that observed with the best available commercial VI improvers.

The excellent performances of some of these polymeric esters as viscosity index improvers for diester synthetic oils are shown in the following Table IV.

TABLE III  
*Qualitative solubilities of synthetic polymers*

| Polymer | Mineral Oil Stocks |                  | Synthetic Oils * |           |                  |                    |
|---------|--------------------|------------------|------------------|-----------|------------------|--------------------|
|         | 70 Pale            | 150 Bright Stock | Diesters         | Silicones | Phosphate Esters | Poly-glycol Esters |
| #1      | S b                | PS               | S                | I         | S                | S                  |
| #2      | PS                 | PS               | S                | I         | S                | S                  |
| #3      | PS                 | I                | S                | I         | S                | S                  |
| #4      | PS                 | PS               | S                | I         | S                | S                  |
| #5      | PS                 | I                | S                | I         | S                | S                  |
| #6      | I                  | I                | PS               | I         | S                | S                  |
| #7      | PS                 | I                | S                | I         | S                | S                  |
| #8      | PS                 | PS               | S                | I         | S                | S                  |

<sup>a</sup> Examples of synthetic oils used for these solubility determinations include: bis(2-ethylhexyl)sebacate, Dow-Corning silicone fluid 200, tricresyl phosphate, and Carbon and Carbide Chemical Company Ucon LB-300.

75 b S= completely soluble, PS= partially soluble, I= insoluble.

TABLE IV

Viscosity index (ASTM D-567) of polymer blends in diester synthetic oils

| Blend                          | Vis. <sup>1</sup> @ 100° F. | Vis. <sup>1</sup> @ 210° F. | V.I. |
|--------------------------------|-----------------------------|-----------------------------|------|
| Diethyl azelate <sup>1</sup>   | 64.0                        | 36.3                        | 136  |
| Plus 1% Polymer #3             | 67.2                        | 36.9                        | 142  |
| Plus 2% Polymer #3             | 70.7                        | 37.6                        | 153  |
| Plus 1% Polymer #4             | 67.5                        | 37.0                        | 145  |
| Plus 2% Polymer #4             | 71.4                        | 38.0                        | 165  |
| Plus 1% Polymer #5             | 73.1                        | 38.3                        | 168  |
| Plus 2% Polymer #5             | 84.8                        | 40.7                        | 186  |
| Plus 3% Polymer #5             | 96.8                        | 42.5                        | 178  |
| Plus 1% Polymer #7             | 71.1                        | 37.7                        | 155  |
| Plus 2% Polymer #7             | 79.1                        | 39.4                        | 182  |
| Plus 1% Polymer #8             | 69.1                        | 37.4                        | 154  |
| Plus 2% Polymer #8             | 74.9                        | 38.9                        | 182  |
| Diethyl sebacate <sup>1</sup>  | 68.4                        | 37.3                        | 152  |
| Plus 1% Polymer #3             | 71.5                        | 37.9                        | 160  |
| Plus 2% Polymer #3             | 74.7                        | 38.7                        | 176  |
| Plus 1% Polymer #5             | 79.9                        | 39.1                        | 168  |
| Plus 2% Polymer #5             | 92.2                        | 41.4                        | 176  |
| Plus 3% Polymer #5             | 105.0                       | 44.1                        | 176  |
| Plus 2% Polymer #7             | 83.3                        | 40.3                        | 183  |
| Dibutyl phthalate <sup>1</sup> | 57.6                        | 33.9                        | 36   |
| Plus 2% Polymer #5             | 72.9                        | 37.0                        | 111  |

<sup>1</sup> The diethyl azelate and diethyl sebacate were the bis(2-ethyl-hexyl) esters of the respective acids; the dibutyl phthalate was di-n-butyl orthophthalate.

<sup>2</sup> Seconds Saybolt Universal.

A most surprising and unexpected finding was the behavior of these polymers in various phosphate ester synthetic oils, where they were not only soluble but displayed remarkable effectiveness in raising the viscosity index. Many phosphate ester oils have excellent lubricity and noninflammability but are notoriously poor in viscosity-temperature characteristics, a shortcoming which has hampered their use; moreover, they are generally incompatible with and hence unresponsive to the commercial viscosity index improvers such as the polyacrylates, polyisobutylenes and polyvinyl ethers. The compatibility and susceptibility to viscosity index improvement which has now been shown to result from the addition of these new polyoxypropylene glycol polyesters to phosphate ester oils serves to broaden the field of usefulness of this class of synthetic oils.

The remarkable ability of these compounds to act as viscosity index improvers is shown by Table V.

TABLE V

Viscosities and viscosity indices of polymer blends in tricresyl phosphate synthetic oil

| 5  | Blend                | Vis. <sup>1</sup> @ 100° F. | Vis. <sup>1</sup> @ 210° F. | V.I. |
|----|----------------------|-----------------------------|-----------------------------|------|
| 10 | Tricresyl phosphate  | 142                         | 39.7                        | -33  |
|    | Plus 1% Polymer #5   | 171                         | 42.2                        | 29   |
|    | Plus 1.5% Polymer #5 | 185                         | 43.4                        | 50   |
|    | Plus 2.0% Polymer #5 | 202                         | 44.8                        | 66   |
|    | Plus 3.0% Polymer #5 | 235                         | 47.5                        | 83   |
|    | Plus 4.0% Polymer #5 | 275                         | 50.9                        | 97   |
|    | Plus 5.0% Polymer #5 | 312                         | 53.9                        | 103  |

<sup>1</sup> Viscosities are seconds Saybolt Universal.

15

Whether diester oils or phosphate ester oils are used, it is not to be understood that the only materials involved are necessarily the oil and my new polyester as a viscosity index improver. As a matter of fact, other materials not only may be present but may be very desirable to prevent oxidation, inhibit rust, and for other reasons. For example, such antioxidants as phenyl alphanaphthylamine, or 2,6-di-tert-butyl para cresol, or polymerized tri-25 methyl dihydroquinoline (sold under the trade-name Age-Rite Resin D) are suitable antioxidants, and other well known antioxidants may also be used. Similarly, any of the well known rust inhibitors or metal deactivators may be used too.

30 Blending of the viscosity index improver with diester and phosphate ester synthetic lubricants may be accomplished by simple mixing. It may be desirable in some instances to prepare a concentrate, because the polyester is viscous and may therefore be inconvenient to handle 35 in some applications. Thus, a small amount of tricresyl phosphate synthetic oil or some suitable diester synthetic oil may be used as the solvent to carry the viscosity index improver into more of the same lubricant. This concentrate can contain anywhere from, say, 5% up to almost 100% of the viscosity-index-improving polyester. The concentrate also may contain any of the antioxidants mentioned above, or others. It may also contain rust inhibitors, metal deactivators, and other materials not incompatible with the lubricant or the polyester.

40 Having given examples and described the principles of 45 the invention, I claim:

1. A lubricant composition consisting essentially of a 50 lubricant selected from the group consisting of diester lubricating oils and phosphate ester lubricating oils, and a sufficient amount to increase appreciably the viscosity index of said lubricant of a polymerized polypropylene glycol ester of an unsubstituted, low molecular weight 55 dibasic organic acid having a glycol-to-acid mol ratio in the range of about 0.875 to 1.111 and having a viscosity of at least 250 centistokes at 210° F. and with at least seven oxypropylene units in the polypropylene glycol radical.

55 2. The composition of claim 1 wherein the ester is



wherein  $n$  averages about 34.

3. The composition of claim 1 wherein the ester is



where  $m$  is about 3 and  $n$  is about 17.

4. The composition of claim 1 wherein the polymerized ester has a viscosity between 250 and 13,000 centistokes at 210° F.

5. The composition of claim 4 wherein the polymerized ester is present in an amount between 1% and 5% of the lubricant.

6. Dioctyl azelate containing between 1% and 5% of



wherein  $n$  averages about 34.

7. Tricresyl phosphate containing an amount sufficient to increase its viscosity index of



wherein  $n$  averages about 34.

8. A new composition of matter having the property of improving the viscosity indices of diester and phosphate ester lubricants, and consisting of a concentrate that consists essentially of up to 95% of a vehicle freely miscible in said lubricant and of more than 5% of a polymer of a polypropylene glycol ester of an unsubstituted low molecular weight dibasic organic acid having a glycol-to-acid mol ratio in the range of about 0.875 to 1.111, said glycol containing at least seven oxypropylene units said polymer having a viscosity of at least 250 centistokes at 210° F.

9. A method of preparing a polymer of a polypropylene glycol ester of an unsubstituted low molecular weight dibasic acid, comprising: refluxing a polypropylene glycol having at least seven oxypropylene units until the water

has been exhaustively removed, and then reacting the glycol with a dibasic acid dichloride in a glycol-to-acid mol ratio in the range between 0.875 and 1.111 in the presence of an HCl acceptor at a temperature in the range between 0° C. and 100° C. said polymer having a viscosity of at least 250° centistokes at 210° F.

References Cited in the file of this patent  
UNITED STATES PATENTS

|           |                 |       |               |
|-----------|-----------------|-------|---------------|
| 2,465,150 | Dickson         | ----- | Mar. 22, 1949 |
| 2,481,372 | von Fuchs       | ----- | Sept. 6, 1949 |
| 2,483,726 | Floyd           | ----- | Oct. 4, 1949  |
| 2,485,376 | Glavis          | ----- | Oct. 18, 1949 |
| 2,562,878 | Blair           | ----- | Aug. 7, 1951  |
| 2,628,974 | Sanderson       | ----- | Feb. 17, 1953 |
| 2,647,885 | Billica         | ----- | Aug. 4, 1953  |
| 2,657,194 | Butler          | ----- | Oct. 27, 1953 |
| 2,820,815 | Matuszak et al. | ----- | Jan. 21, 1958 |
| 2,837,562 | Matuszak et al. | ----- | June 3, 1958  |
| 2,929,786 | Young et al.    | ----- | Mar. 22, 1960 |

OTHER REFERENCES

"Experiments in Organic Chemistry," by Fieser, 2nd Edition, 1941, D. C. Heath & Co., p. 398.